

Dec. 20, 1927.

1,653,344

M. S. CLAWSON

CASTING MOLD AND METHOD OF MAKING SAME

Filed April 7, 1921



Inventor

Monroe S. Clawson

By D. A. Gourick

Attorney

Witness:

J. Milton Fester

## UNITED STATES PATENT OFFICE.

MONROE S. CLAWSON, OF UPPER MONTCLAIR, NEW JERSEY.

## CASTING MOLD AND METHOD OF MAKING SAME.

Application filed April 7, 1921. Serial No. 459,318.

This invention relates to the metallurgical art, particularly to molds and casting processes, and has for its object the provision of a novel mold adapted for use in the casting of high speed steels and other metals, and particularly those alloys that are readily oxidizable, the mold being of such a nature as to withstand the very high temperatures necessary in the fusing of such metals or alloys without breaking down, the mold being furthermore of such a nature as to be very porous so that when used in carrying out my process which involves the application of suction upon the mold or impression, the gases generated at the surface of contact of the molten material with the mold will be drawn off in order to prevent the formation of blisters, air holes, and what is known in the art as "minus material".

An important object is the provision of a mold of this character consisting of high refractory material containing an excess of oil or varnish whereby to present a smooth molding surface to the molten metal while retaining sufficient porosity to facilitate the exhaust or drawing off of the gases generated when the metal is poured, the mold being also of such a tenacious formation as to permit machining thereof whereby to define a sharp impression when the metal is cast therein.

I am aware that the art of casting with suction applied to the mold is not broadly new and I am also aware that oil and sand have been used in the formation of molds, the oil being either of a mineral or vegetable type. I am also aware that certain of the ingredients which I employ in the composition of my mold have been used before in the same art but heretofore it has apparently been impossible to make a mold containing oil adapted for use in casting high speed steels or other alloys containing magnesium, tungsten or other readily oxidizable metals owing to the fact that the molds known and used break up when subjected to exposure to the high temperatures necessary to the fusing of such alloys. Such well known molds either disintegrate to a greater or less extent and cause rough castings or else the oil used as a binder gasifies to such an extent as to cause too great a number of blow holes, blisters and the like which render the casting practically worthless.

It is to avoid the above mentioned objections that the present invention has been de-

signed, this invention insuring the production of smooth castings even from delicate or intricate mold impressions.

In carrying out my invention I provide a mold formed of a refractory material, preferably a metal oxide, such as oxide of silicon, magnesium, aluminum, calcium, or even others such as iron, zirconium, thorium, cerium and many others. Whichever oxide is used is mixed with a fatty or hydrocarbon binder such as a drying oil or varnish, the proportions of oxide and binder varying under different conditions though it is necessary to use what I may term an excess of the oil or varnish. The impression is made in this mass in the customary manner and the mold is then baked by suitable means and at a suitable temperature to render it solid.

The exact length of time during which the mold is baked may of course vary, depending upon the proportion of oxide and drying material, and also depending upon the temperature and other conditions. However, the intention is to discontinue the baking before the mold becomes dry and brittle. If an excess of oil or other drying material is used the baking may be continued for as long a time as ordinary molds are baked but would still retain sufficient of the oil to be very slightly plastic, in the sense of being indentable if struck by a hard object though not being brittle or friable. The mold is, however, porous so as to permit suction through it. The condition is of course sufficiently hard to prevent any possible distortion when molten metal is poured into the mold. It is intended that sufficient oil remain in the mold after the baking operation to necessitate suction for carrying off the gases formed by the burning of the oil when the metal impinges against the mold.

In carrying out the process it is of course necessary to provide some apparatus in which suction may be applied to the mold. Such an apparatus is conventionally illustrated in the drawing which shows a longitudinal sectional view through a suitable holder or receptacle 10, naturally of refractory material, provided at its bottom with an outlet tube 11 to which suction is applied by any suitable means such as an air pump or the like, not shown. The mold or impression, designated by the numeral 12, which is formed from the above described mass, is

placed within this receptacle 10 and the molten metal is poured onto the mold. The mold, when in position within its holder, really acts as a diaphragm and it is to be observed that the tube to which suction is applied is located below the mold. When the molten metal is poured onto the mold 12 suction is applied to the tube 11 so that the gases generated by the burning or disintegration of the excess oil in the mold may be sucked out through the pores of the mold whereby to prevent the formation of air holes, blisters, and the like in the resultant casting 13 and to insure the drawing of the molten metal into even the smallest indentations in the mold. This will insure a sharp casting.

It will be noted that there is no intention of rarefying the air within the mold holder or receptacle, but that absolutely direct suction through the mold is produced to carry away or exhaust the hydrocarbon, carbon monoxide and oxy-hydrogen gases caused by the disintegration of the binder at the surface of contact of the molten metal with the mold. It is strictly the diaphragm-like nature of the mold which permits this action.

In actual practice I have discovered that a mold constructed of the above mentioned materials and treated as described, is not only capable of being carved or machined to produce sharp impressions but is also capable of withstanding the high temperatures necessary to cause fusing of the many alloys incapable of being properly cast with the ordinary apparatus and in the ordinary processes. I have ascertained from experiment that with my mold and process it is possible to cast alloys of steel, nickel, cobalt, and the like in intricate shapes to almost exact size. In my process I entirely avoid the formation of what is known in the art as a "skin" on the surface of the casting unlike the internal structure of the metal itself, such skin being caused by the "burning in" of some of the molding material and the chilling caused by the binder used to maintain the shape of the article to be cast. In casting alloys requiring a high temperature to effect melting thereof, the ordinary mold materials such as plaster of Paris depending upon water of crystallization, are unsuitable as such a mold breaks down at a low tem-

perature. In my mold, however, I have discovered that all the above enumerated disadvantages have been eliminated so that almost perfect castings of substantially exact size can be easily produced.

While I have shown and described the preferred embodiment of my invention, it is of course to be understood that I reserve the right to make such changes in the form, construction and arrangement of parts as will not depart from the spirit of the invention or the scope of the subjoined claims.

Having thus described my invention, I claim:

1. A mold consisting of an oxide mixed with drying oil and baked to machinable hardness with an excess of oil remaining in the mold whereby to necessitate suction during casting for removing mixed gases formed by the disintegration of the oil upon impingement of molten metal against the mold.

2. The method of making a mold consisting in mixing together a mineral oxide and a fluent drying material, baking the mold to substantial hardness and discontinuing the baking at a point where sufficient fluent drying material remains in the mold to impart a slight but appreciable plasticity thereto and to require suction during casting.

3. The method of making a mold, consisting in mixing together a metallic oxide and a drying oil, making the impression in the mass, and baking the mold to expel the major portion of the oil and to bring about substantial hardness and porosity, the baking being discontinued at a point where sufficient oil remains in the mold to necessitate suction during casting.

4. A mold consisting of a mineral oxide and a fluent drying material treated to possess machineable hardness and to retain a sufficient quantity of the drying material after treatment to possess malleability.

5. A mold comprising a mineral oxide and a resinous drying material of fluent character, the mold being baked to machineable hardness, and having sufficient drying material remaining after treatment to render it malleable and to require suction during casting for the carrying off of gases caused by disintegration of the drying material.

In testimony whereof I hereto affix my signature.

MONROE S. CLAWSON.